

## 1

3,418,111

**COBALT BASE ALLOY**

Robert B. Herchenroeder, Kokomo, Ind., assignor to  
 Union Carbide Corporation, a corporation of New  
 York  
 No Drawing. Filed Oct. 27, 1966, Ser. No. 589,822  
 3 Claims. (Cl. 75—171)

This invention relates to cobalt base alloys. More particularly, this invention relates to cobalt-chromium-tungsten-nickel alloys containing relatively small amounts of lanthanum which are characterized by improved oxidation resistance at high temperatures in addition to having excellent high temperature mechanical properties.

Cobalt base alloys have been used extensively in the past for high temperature applications and have been found to be generally satisfactory except that in some instances they have been lacking in oxidation resistance, when compared to nickel base alloys. However, at high temperatures, on the order of 1800 to 2100° F. nickel base alloys have limited mechanical properties. Accordingly, it would represent an advance in the art if cobalt base alloys could be provided with oxidation resistance comparable to or better than that of nickel base alloys at high temperatures, while retaining the characteristic strength and mechanical properties of cobalt base alloys at high temperatures.

It is therefore an object of the present invention to provide a cobalt base alloy having improved oxidation resistance at elevated temperatures.

It is another object of the present invention to provide a cobalt base alloy having excellent high temperature mechanical properties and additionally having improved oxidation resistance.

Other objects will be apparent from the following description and claims.

A cobalt base alloy in accordance with the present invention is an alloy consisting essentially of about

|                                 | Percent   |
|---------------------------------|-----------|
| Chromium                        | 18-30     |
| Tungsten                        | 8-18      |
| Iron                            | Up to 10  |
| Carbon                          | 0.01-0.35 |
| Nickel                          | 8-30      |
| Silicon                         | Up to 1   |
| Lanthanum                       | 0.02-0.2  |
| Cobalt, balance to 61% maximum. |           |

wherein the

$$\frac{\text{percent Cr} + \text{percent W}}{\text{percent C}}$$

ratio in the alloy is at least about 110, with an alloy having a ratio of less than about 200 containing at least about 0.2% silicon.

A preferred range of the alloy of the present invention is as follows:

|                                 | Percent   |
|---------------------------------|-----------|
| Chromium                        | 19-28     |
| Tungsten                        | 12-18     |
| Iron                            | Up to 5   |
| Carbon                          | 0.01-0.15 |
| Nickel                          | 10-25     |
| Silicon                         | Up to 0.6 |
| Lanthanum                       | 0.02-0.15 |
| Cobalt, balance to 61% maximum. |           |

Alloys in the foregoing range have been found to have an optimum combination of oxidation resistance and mechanical properties at high temperatures.

## 2

In addition to the specifically mentioned alloy constituents, other metals can be adventitiously present in the alloy of this invention in minor amounts. For example, zirconium may be present in amounts up to about 2%; vanadium up to about 2%; up to about 1% beryllium; boron up to about 0.02%; manganese up to about 2%; Ti+Al up to about 4%; Ta+Cb up to about 8%.

It has been discovered, as part of the present invention that with alloy compositions as described above, a relatively small lanthanum addition provides remarkable oxidation resistance at high temperatures when the critical and defined relationship between chromium, tungsten, carbon and silicon is observed.

It has also been discovered that other rare earth metals can be present with the lanthanum, such as occurs when mischmetal is used to introduce lanthanum, without detrimentally effecting the improved oxidation resistance. However, the presence of other rare earth metals, in an aggregate amount exceeding the lanthanum content, results in the formation of stringers and non-metallic inclusions in the alloy which adversely affect its weldability and result in low strength welds. Consequently, for alloys intended for welding applications, the lanthanum is preferably added in essentially elemental form, and should, in any event, exceed the aggregate amount of other rare earth metals in the final alloy. For alloys which are not intended for welding, however, the lanthanum addition can be made using any convenient technique such as mischmetal, elemental lanthanum or lanthanum containing alloys.

Table I shows alloy compositions which have been prepared by being melted, cast into ingots of about 20-25 lbs., forged to plate about  $\frac{1}{2}$  to  $\frac{3}{4}$  inch thick, hot rolled to sheet and annealed at 2100-2250° F. for 10-15 minutes and quenched. The lanthanum additions to alloys K and L were made in the form of mischmetal and for the other lanthanum-containing alloys the addition was made using either elemental lanthanum or lanthanum-cobalt alloy containing about 20% lanthanum.

Specimens of the various alloys of Table I, in sheet form  $\frac{3}{4}$  inch x  $\frac{3}{4}$  inch x 0.06-0.125 inch thick, were tested for oxidation resistance and the results are shown in Table II.

The procedure for the oxidation tests to which the alloy specimens were subjected was as follows:

One hundred hour continuous oxidation test.

(1) Prepare specimen by grinding all surfaces to a 120 grit finish.

(2) Measure the surface area of specimen and weight.

(3) Expose the specimen at 2000° F. continuously for 100 hours in dry flowing air (2 cubic feet per hour).

(4) Air cool the sample.

(5) Descale the sample in a salt bath.

(6) Carefully weigh the descaled sample and calculate the weight loss.

(7) Calculating the depth of penetration per year of exposure follows:

$$\frac{\text{Weight loss}}{\text{density}} \times \frac{1}{\text{area of sample}} \times \frac{100 \text{ hours}}{\text{hours/year}}$$

An intermittent oxidation test is similar except that instead of exposing the sample 100 hours continuously the sample is exposed for eight three-hour periods, and then for four nineteen-hour periods. The sample is allowed to cool at room temperature between each period.

TABLE I

| Alloy | Cr    | W     | Fe   | C    | Ni    | Mn   | B     | Si   | Al    | La    | Co                |
|-------|-------|-------|------|------|-------|------|-------|------|-------|-------|-------------------|
| A     | 19.42 | 12.68 | 2.15 | 0.10 | 19.40 | 0.56 | 0.005 | 0.01 | 0.08  | 0.04  | Bal.              |
| B     | 21.89 | 14.02 | 2.43 | 0.12 | 19.48 | 0.64 | 0.015 | 0.08 | 0.28  | 0.05  | Bal.              |
| C     | 19.49 | 14.64 | 2.01 | 0.09 | 10.41 | 1.30 | 0.003 | 0.14 | ----- | 0.13  | Bal. <sup>1</sup> |
| D     | 19.65 | 12.28 | 2.38 | 0.29 | 19.20 | 0.72 | 0.013 | 0.32 | ----- | 0.09  | Bal.              |
| E     | 22.30 | 14.75 | 1.43 | 0.09 | 18.80 | 0.66 | 0.016 | 0.11 | 0.18  | 0.12  | Bal.              |
| F     | 23.03 | 14.48 | 1.88 | 0.11 | 25.30 | 0.54 | 0.012 | 0.01 | 0.18  | 0.08  | Bal.              |
| G     | 22.44 | 14.81 | 1.30 | 0.09 | 18.88 | 0.56 | 0.018 | 0.1  | 0.20  | 0.13  | Bal.              |
| H     | 22.94 | 14.55 | 1.18 | 0.11 | 18.88 | 0.56 | 0.016 | 0.19 | 0.18  | 0.10  | Bal.              |
| I     | 27.74 | 17.66 | 1.38 | 0.12 | 23.16 | 0.67 | 0.021 | 0.17 | 0.28  | 0.04  | Bal.              |
| J     | 22.98 | 14.88 | 1.23 | 0.10 | 19.32 | 0.56 | 0.018 | 0.21 | 0.30  | 0.04  | Bal.              |
| K     | 25.63 | 12.62 | 2.35 | 0.10 | 18.44 | 0.44 | 0.005 | 0.03 | 0.13  | 0.02  | Bal. <sup>2</sup> |
| L     | 25.63 | 12.62 | 2.35 | 0.10 | 18.44 | 0.44 | 0.005 | 0.03 | 0.13  | 0.04  | Bal. <sup>3</sup> |
| M     | 22.71 | 14.47 | 1.35 | 0.10 | 19.20 | 0.64 | 0.013 | 0.06 | 0.15  | 0.06  | Bal.              |
| N     | 22.57 | 14.50 | 2.48 | 0.08 | 19.24 | 1.10 | 0.016 | 0.03 | 0.21  | 0.08  | Bal.              |
| O     | 22.46 | 14.39 | 3.30 | 0.07 | 19.08 | 1.06 | 0.016 | 0.05 | 0.18  | 0.05  | Bal.              |
| P     | 22.30 | 14.38 | 3.25 | 0.06 | 18.88 | 1.90 | 0.016 | 0.04 | 0.13  | 0.04  | Bal.              |
| Q     | 23.34 | 12.35 | 2.58 | 0.12 | 19.60 | 0.88 | 0.001 | 0.64 | 0.23  | 0.06  | Bal.              |
| R     | 23.24 | 13.42 | 1.65 | 0.11 | 20.76 | 0.42 | 0.001 | 0.31 | ----- | 0.03  | Bal.              |
| S     | 21.56 | 13.43 | 1.43 | 0.13 | 21.80 | 0.36 | 0.003 | 0.26 | 0.33  | 0.06  | Bal.              |
| T     | 19.42 | 12.68 | 2.15 | 0.10 | 19.40 | 0.56 | 0.005 | 0.01 | 0.08  | ----- | Bal.              |
| U     | 19.88 | 13.00 | 1.68 | 0.30 | 19.20 | 0.64 | 0.018 | 0.08 | ----- | ----- | Bal.              |
| V     | 19.88 | 13.00 | 1.68 | 0.29 | 19.20 | 0.64 | 0.018 | 0.08 | 0.08  | 0.05  | Bal.              |
| W     | 21.89 | 14.02 | 2.43 | 0.11 | 19.48 | 0.64 | 0.015 | 0.08 | 0.28  | ----- | Bal.              |
| X     | 20.02 | 14.84 | 1.85 | 0.10 | 10.40 | 1.46 | 0.009 | 0.05 | 0.05  | ----- | Bal.              |

<sup>1</sup> 0.47 Mo.<sup>2</sup> Total rare earth content=0.08%.<sup>3</sup> Total rare earth content=0.34%.

TABLE II.—OXIDATION RATE IN MILS PER YEAR

| Alloy             | Continuous<br>2,000° F. | Intermittent<br>2,000° F. |
|-------------------|-------------------------|---------------------------|
| A                 | 20                      | 33                        |
| B                 | -----                   | 20                        |
| C                 | 9                       | 15                        |
| D                 | 23                      | 24                        |
| E                 | 7                       | 14                        |
| F                 | 13                      | 8                         |
| G                 | 10                      | 23                        |
| H                 | 12                      | 19                        |
| I                 | 13                      | 17                        |
| J                 | 12                      | 18                        |
| K                 | 13                      | 14                        |
| L                 | 9                       | 12                        |
| M                 | 22                      | 9                         |
| N                 | 12                      | 13                        |
| O                 | 17                      | 19                        |
| P                 | 14                      | 14                        |
| Q                 | 11                      | 10                        |
| R                 | 14                      | 15                        |
| S                 | 7                       | 7                         |
| T                 | 23                      | 39                        |
| U                 | -----                   | 179                       |
| V                 | 25                      | 283                       |
| W                 | 23                      | 47                        |
| X                 | 31                      | 143                       |
| Hastelloy alloy X | -----                   | 21                        |

As can be seen from Table II, alloys A through S, which contain lanthanum and are within the scope of the present invention, have superior oxidation properties as compared to alloys T through X, which while generally similar in composition, are outside of the compositional limits of this invention. Alloys T, U, W and X, for example, do not contain lanthanum and can be seen to be considerably less oxidation resistant, particularly under intermittent conditions, than alloys in the group A through S of similar composition but which additionally contain a lanthanum addition. Alloy V, while containing lanthanum, does not have a sufficiently high



ratio, and is characterized by very poor oxidation resistance under intermittent conditions.

Hastelloy Alloy X<sup>1</sup>, a widely used nickel base alloy (nominal composition: 22% Cr, 1% W, 9% Mo, 18% Fe, 0.1% C, 2.5% max. Co, Ni bal.), generally considered to be the industry standard for oxidation resistance, was also tested under intermittent conditions and the result recorded in Table II to show the significance of the improved oxidation resistant properties of the cobalt base alloys of this invention.

Alloy S (AIM composition: 21-22% Cr, 13-14% W, 1-2% Fe, 22% Ni, 0.3% Si, 0.1% C, 0.06% La, balance Co) can be seen from Table II to have exceptional oxidation resistance under continuous and intermittent condi-

tions and is a particularly preferred alloy of the present invention.

As shown by the test data of Table III, alloys of this invention, in addition to having improved oxidation resistance, are also characterized by excellent mechanical properties at high temperatures. It can also be seen from Table III that the alloys of the present invention, which exhibited oxidation resistance comparable to Hastelloy Alloy X, have much better mechanical properties particularly at higher temperatures.

TABLE III

| Alloy                | 0.2% offset<br>yield strength,<br>K p.s.i. |           | Ultimate<br>tensile strength,<br>K p.s.i. |           | Elongation,<br>percent |           |
|----------------------|--------------------------------------------|-----------|-------------------------------------------|-----------|------------------------|-----------|
|                      | 1,600° F.                                  | 2,000° F. | 1,600° F.                                 | 2,000° F. | 1,600° F.              | 2,000° F. |
| A                    | 36.1                                       | 8.4       | 61.8                                      | 16.3      | 51                     | 52        |
| B                    | 31.0                                       | 9.6       | 62.1                                      | 16.1      | 41                     | 30.1      |
| C                    | 32.7                                       | -----     | 73.8                                      | -----     | 49                     | -----     |
| D                    | 41.6                                       | -----     | 66.3                                      | -----     | 53                     | -----     |
| E                    | 14.6                                       | -----     | 23.0                                      | -----     | 66.2                   | -----     |
| F                    | 13.8                                       | -----     | 21.1                                      | -----     | 50.7                   | -----     |
| G                    | 14.9                                       | -----     | 23.5                                      | -----     | 56.2                   | -----     |
| H                    | 15.5                                       | -----     | 25.5                                      | -----     | 58.4                   | -----     |
| I                    | 16.3                                       | -----     | 25.1                                      | -----     | 64.8                   | -----     |
| K                    | 39.9                                       | 12.8      | 58.8                                      | 20.8      | 44                     | -----     |
| L                    | 38.7                                       | 12.0      | 61.8                                      | 20.6      | 54.8                   | 38.9      |
| M                    | 14.6                                       | -----     | 24.6                                      | -----     | 57.6                   | -----     |
| N                    | 14.6                                       | -----     | 22.6                                      | -----     | 56.4                   | -----     |
| O                    | 15.0                                       | -----     | 23.9                                      | -----     | 57.2                   | -----     |
| P                    | 15.8                                       | -----     | 24.1                                      | -----     | 69.2                   | -----     |
| Q                    | 18.3                                       | -----     | 29.2                                      | -----     | 41.5                   | -----     |
| Hastelloy<br>alloy X | 25.7                                       | 8.0       | 36.5                                      | 13        | 50                     | 40        |

What is claimed is:

1. An alloy characterized by improved resistance to oxidation at elevated temperatures consisting essentially in weight per cent of about:

|                                 | Percent   |
|---------------------------------|-----------|
| Chromium                        | 18-30     |
| Tungsten                        | 8-18      |
| Iron                            | Up to 10  |
| Carbon                          | 0.01-0.35 |
| Nickel                          | 8-30      |
| Silicon                         | Up to 1   |
| Lanthanum                       | 0.02-0.2  |
| Cobalt, balance to 61% maximum. | -----     |

wherein the

$$\frac{\text{percent Cr} + \text{percent W}}{\text{percent C}}$$

ratio in the alloy is at least about 110, with an alloy having a ratio of less than about 200 containing at least about 0.2% silicon.

<sup>1</sup> Trademark of Union Carbide Corporation.

2. An alloy in accordance with claim 1 consisting essentially of about:

|                                 | Percent   |
|---------------------------------|-----------|
| Chromium                        | 19-28     |
| Tungsten                        | 12-18     |
| Iron                            | Up to 5   |
| Carbon                          | 0.01-0.15 |
| Nickel                          | 10-25     |
| Silicon                         | Up to 0.6 |
| Lanthanum                       | 0.02-0.15 |
| Cobalt, balance to 61% maximum. |           |

3. An alloy in accordance with claim 1 consisting essentially of about:

|          | Percent |    |
|----------|---------|----|
| Chromium | 21-22   | 15 |
| Tungsten | 13-14   |    |

|           |       |         |
|-----------|-------|---------|
| Iron      | ----- | 1-2     |
| Carbon    | ----- | 0.1     |
| Nickel    | ----- | 22      |
| Silicon   | ----- | 0.3     |
| Lanthanum | ----- | 0.06    |
| Cobalt    | ----- | Balance |

#### References Cited

#### UNITED STATES PATENTS

|    |           |        |               |       |        |
|----|-----------|--------|---------------|-------|--------|
| 10 | 2,075,718 | 3/1937 | Hessenbruch   | ----- | 75-171 |
|    | 2,744,010 | 5/1956 | Callaway      | ----- | 75-171 |
|    | 2,746,860 | 5/1956 | Binder et al. | ----- | 75-171 |
|    | 3,304,176 | 2/1967 | Wlodek        | ----- | 75-171 |
|    | 3,366,478 | 1/1968 | Wheaton       | ----- | 75-171 |

RICHARD O. DEAN, Primary Examiner.